

Dec. 5, 1950

B. A. FRIES

2,532,490

PROCESS FOR RECOVERY OF C<sup>14</sup> ACTIVITIES

Filed Sept. 28, 1948



INVENTOR.  
BERNARD A. FRIES

BY

*P. A. Anderson*

ATTORNEY.

## UNITED STATES PATENT OFFICE

2,532,490

PROCESS FOR RECOVERY OF C<sup>14</sup> ACTIVITIES

Bernard A. Fries, El Cerrito, Calif., assignor to  
the United States of America as represented by  
the United States Atomic Energy Commission

Application September 28, 1948, Serial No. 51,623

16 Claims. (Cl. 23—209)

1

This invention relates to processes for the recovery of C<sup>14</sup> and, more particularly, to the improvements in processes for the recovery of C<sup>14</sup> activities from irradiated metal nitrides.

The nuclear reaction represented by the equation N<sup>14</sup>(n,p)C<sup>14</sup> has been known for some time. In the practical process for producing C<sup>14</sup>, from N<sup>14</sup>, a suitable chemical compound of nitrogen is irradiated with neutrons. Several properties are desirable in a compound which is to be so irradiated. The compound should be a stable solid, it should contain a large proportion of nitrogen, the constituents other than nitrogen should have a low capture cross section for neutrons, the compound should be free of normal carbon contamination, and the compound should be readily soluble or decomposable to facilitate release of the C<sup>14</sup> activities. Metallic nitrides have been found to possess these desired properties to a high degree. In carrying out the process of irradiation, metallic nitride is sealed in an aluminum container and the container containing the nitride is subsequently placed in a uranium neutron reactor. After the required period of exposure, the nitride in the sealed container is removed from the reactor. The C<sup>14</sup> product activities are contained in the much larger quantity of unreacted nitride as a variety of simple carbon compounds. Older methods for recovering the C<sup>14</sup> activities utilized an alkaline dissolution step followed by an alkaline solution-oxidation step to release the activities. This alkaline process suffers from several serious faults. These faults are that large amounts of ammonia gas are released with almost explosive violence during the reaction of the nitride with alkali and that disproportionately large amounts of oxidant are consumed in the solution-oxidation step.

Now, it has been found that the difficulties attached to the operation of the alkaline process may be avoided by utilizing an acidic dissolution step followed by an acidic solution-oxidation step. Furthermore, it has been found that product fractions having highly enhanced specific activity may be obtained by following certain sequences of operations in the procedures.

Accordingly, it is an object of this invention to release C<sup>14</sup> activities from irradiated metal nitrides by reaction with acid.

It is another object of this invention to utilize acidic solution-oxidation to release C<sup>14</sup> activities from solutions produced by the reaction of irradiated metal nitrides with acid.

It is another object of this invention to remove

2

C<sup>14</sup> activities, which are released by acidic reaction and solution-oxidation, from the reaction site, by entrainment in a gaseous stream.

It is a further object of this invention to recover C<sup>14</sup> activities, which are entrained in a gaseous stream, by absorption.

It is another object of this invention to recover C<sup>14</sup> activities which are not absorbable by subjecting the gaseously entrained activities to combustion and subsequent absorption.

It is another object of this invention to provide operational sequences which yield product fractions of enhanced specific activities.

The invention, both as to its organization and method of operation, together with further objects and advantages thereof, will best be understood by reference to the following specification taken in connection with the accompanying drawing, in which the single figure is a schematic illustration of apparatus suitable for carrying out the processes of the present invention.

In accordance with the present invention, a charge of irradiated metal nitride is placed in a reaction vessel which is provided with heating and stirring means, means for introducing reagents, and means for introducing a gaseous stream for entraining released C<sup>14</sup> activities. The reaction vessel is followed in sequence by a stripping condenser column, a first absorber, a combustion reactor, and a second absorber.

The nitride is then reacted with a mineral acid and heated while a slow stream of gas sweeps the system. Later a solution oxidant is added to the reaction mixture, and the boiling and sweeping is continued.

The product may be collected as a single mass by eliminating the first absorber from the train of apparatus, but it has been found that by utilizing dual absorbers during the period of heating with acid and a fresh second absorber and no first absorber during the period of heating which follows the addition of solution-oxidant, the product may be resolved into fractions of which some possess enhanced specific activity.

Now consider the materials which may be treated by this process. All metallic nitrides are not of equal suitability for being irradiated with neutrons. In addition to the properties which are mentioned above as being desirable in a nitride, another extremely important property to be taken into consideration is that of relative neutron capture cross section. It is desirable that the metallic component of the nitride have low capture cross section for neutrons. The nitrogen capture cross section for slow neutrons is

of the order of 1.7 barns. The limit of relative neutron capture cross section for the metallic component is of the order of tenfold this value, or for convenience, the value of approximately 20 barns. Of course, it is the relative absorption value derived from atomic ratio and capture cross section of each component which must be employed in making the determination. A list of suitable nitrides, together with the relative capture cross section of the components, is shown in Table 1.

Table 1

| Chem. formula of nitride       | Absorp. cross section of N (relative) | Absorp. cross section of metallic component (relative) | Relative absorb. ratio |
|--------------------------------|---------------------------------------|--------------------------------------------------------|------------------------|
| Be <sub>3</sub> N <sub>2</sub> | 2 X 1.7                               | 3 X 0.01                                               | 0.009                  |
| Na <sub>3</sub> N              | 1 X 1.7                               | 3 X 0.45                                               | 0.8                    |
| Mg <sub>3</sub> N <sub>2</sub> | 2 X 1.7                               | 3 X 0.35                                               | 0.3                    |
| AlN                            | 1.7                                   | 1.7                                                    | 0.24                   |
| Si <sub>3</sub> N <sub>4</sub> | 4 X 1.7                               | 3 X 0.22                                               | 0.66                   |
| K <sub>3</sub> N               | 1.7                                   | 3 X 2.5                                                | 7.5                    |
| Ca <sub>3</sub> N <sub>2</sub> | 2 X 1.7                               | 3 X 0.45                                               | 0.4                    |
| TiN                            | 1.7                                   | 1.7                                                    | 5.5                    |
| VN                             | 1.7                                   | 1.7                                                    | 6.0                    |
| CrN                            | 1.7                                   | 1.7                                                    | 3.0                    |
| Fe <sub>2</sub> N              | 1.7                                   | 2 X 2.5                                                | 5.0                    |
| Fe <sub>3</sub> N              | 1.7                                   | 4 X 2.5                                                | 10.0                   |
| Os <sub>3</sub> N              | 1.7                                   | 3 X 3.5                                                | 10.5                   |
| Zn <sub>3</sub> N <sub>2</sub> | 2 X 1.7                               | 3 X 1.2                                                | 1.0                    |
| GaN                            | 1.7                                   | ca. 2.0                                                | 1.0                    |
| CbN                            | 1.7                                   | less than 1.0                                          | less than 0.5          |

The tabulated list indicates a series of nitrides which are suitable from the neutron capture standpoint and which, it is believed, may be treated successfully by applicant's process. This list is not considered a complete tabulation of all possible satisfactory nitrides but is intended merely as an illustration of a suitable method of differentiating the applicability of any particular nitride. It will be noted that considerable variation exists in the neutron capture values, and it will be further noted that the compounds Be<sub>3</sub>N<sub>2</sub>, Na<sub>3</sub>N, AlN, Si<sub>3</sub>N<sub>4</sub>, Mg<sub>3</sub>N<sub>2</sub>, Ca<sub>3</sub>N<sub>2</sub>, Zn<sub>3</sub>N<sub>2</sub>, GaN, and CbN have a relative absorption ratio

$$\left( \frac{\sigma}{\sigma} \right)_{\text{Nitride}}$$

of about one or less than one. These nitrides may be considered to be a preferred class.

For the practical operation of the process, beryllium nitride was chosen from the preferred class as a nitride which possesses properties that fulfill the irradiation requirements. This nitride was found to be entirely satisfactory from the process viewpoint.

The reagents utilized in the process are as follows: Sulfuric acid was selected as a mineral acid possessing properties easily adaptable to utilization in this process. It is required that the acid be strongly acidic, relatively nonvolatile, and contain no normal carbon contamination. Several of the other mineral acids may be utilized with modification of the process.

The solution-oxidant employed in this process was chromium-trioxide (Cr<sub>2</sub>O<sub>3</sub>) and was found entirely satisfactory. The property required of an oxidant in this process is that it must be capable of oxidizing carbon compounds in solution.

The absorbing medium utilized is normally 1 N sodium hydroxide solution. The equivalents of this material are to be found in the group of materials which produce alkaline solutions or the group which yield solutions from which insoluble carbonate may be precipitated.

Now with reference to the attached schematic drawing comprising a single figure, there will be

described a suitable apparatus for conducting the operations of the processes of this invention. The apparatus may be seen to comprise a reaction vessel 1, a stripping (reflux) condenser column 2, alkaline absorber 3, combustion reactor 4, and alkaline absorber 5, connected in sequence. Reaction vessel 1 is fitted with heating means 6, mechanical stirring means 7, solid reagent introducing means 8, fluid reagent introducing means 9, and gas introducing means 11. Stripping condenser 2 is connected to the exit of reaction vessel 1 for the purpose of removing entrained aqueous and acidic components from the gaseous sweep. Absorber 3 is of the bubble type containing an absorbing medium. Absorber 3 may be omitted from the train of apparatus by opening valve 12 and closing valves 13 and 14. Combustion reactor 4 is of the normal copper oxide type used in the combustion of carbonaceous materials. Absorber 5 is similar to absorber 3. The gaseous sweep is vented to the atmosphere after passage through absorber 5.

In accordance with the invention, a charge of irradiated nitride is placed in reaction vessel 1. A slow stream of nitrogen or other inert gas is introduced to entrain the carbon compounds released in the reaction. A stream of inert gas is utilized during the early stages of the process to eliminate hazard from explosions of hydrogen which may be generated if beryllium metal is present in the nitride. 10 ml. of water for each gram of nitride is then added to the nitride, and the mixture is brought to a slow boil with constant stirring. 8 ml. of 18 N sulfuric acid per gram of nitride is now added to the boiling slurry. When the reaction appears complete, the nitrogen sweep is replaced by a stream of oxygen, sufficient acid is added to make the solution 6 N in H<sub>2</sub>SO<sub>4</sub>, and boiling and sweeping is continued for 16 to 24 hours. At the end of that time, absorber 3 is bypassed as described above, absorber 5 is emptied and refilled with fresh absorbing medium, and the solution is made 0.2 M. in Cr<sub>2</sub>O<sub>3</sub>. The solution is then boiled and swept with oxygen for a period of 16 to 24 hours. In this mode of operation, three fractions of product are collected; the first, in absorber 3 during the first period of operation; a second, in absorber 5 during the first period of operation; and a third, in absorber 5, during the second period of boiling and sweeping.

The collection of the various fractions is made possible by the difference in chemistry of the carbon compounds found in the solution which results from reaction of the nitride with acid. The compounds found on acidic dissolution of irradiated nitrides are CH<sub>4</sub>, CO, CO<sub>2</sub>, HCN, HCOOH, CH<sub>3</sub>OH, and HCHO. The CO<sub>2</sub>, HCN, CH<sub>4</sub>, and CO are removed from the solution during the first period of operation. The CO<sub>2</sub> and HCN are collected in absorber 3, and the CH<sub>4</sub> and CO are collected in absorber 5 during the first period of operation. The HCOOH, HCHO, and CH<sub>3</sub>OH are released during the second period of operation by the solution oxidation and are collected in absorber 5. In some cases, carriers are added to the solution to effect complete recovery. The CO<sub>2</sub> and HCN fraction may be further resolved by precipitating the CO<sub>2</sub> as carbonate and the HCN by means of silver. The carbonate and cyanide precipitates may then be burned and collected are separate fractions of carbonate.

All of the C<sup>14</sup> may thus be collected as carbonate fractions in alkaline absorbers and may be removed from the absorbing solution by pre-

cipitation, as with barium. The precipitated  $\text{BaCO}_3$  may be separated from the solution by filtering and drying. This product  $\text{BaCO}_3$ , or more properly  $\text{BaC}^{14}\text{O}_3$  may be used as a source of  $\text{C}^{14}$  for the synthesis of  $\text{C}^{14}$  compounds.

Examples of the results obtained in operating this process follow. The assay of the samples was done by means of electronic counting apparatus which employed a thin mica window counting chamber.

#### EXAMPLE I

##### $\text{C}^{14}$ recovered from a 5.12 gm. sample of irradiated $\text{Be}_3\text{N}_2$

| Origin of Fraction      | Product as $\text{BaCO}_3$ , mg. | Specific Activity, c./m./mg. of $\text{BaCO}_3$ | Total $\text{C}^{14}$ , c./m. |
|-------------------------|----------------------------------|-------------------------------------------------|-------------------------------|
| $\text{CO}_2^1$         | 146.2                            | $2.02 \times 10^6$                              | $2.95 \times 10^5$            |
| $\text{HCN}^2$          | 431                              | $1.19 \times 10^4$                              | $5.12 \times 10^5$            |
| $\text{CH}_4\text{-CO}$ | 500.4                            | $9.39 \times 10^4$                              | $4.69 \times 10^5$            |
| Oxidizable <sup>3</sup> | 126.6                            | $1.45 \times 10^5$                              | $1.84 \times 10^5$            |
| Cleanup <sup>4</sup>    | 145.8                            | $5.42 \times 10^3$                              | $7.91 \times 10^5$            |

<sup>1</sup>  $\text{Na}_2\text{CO}_3$  carrier was added at the time of precipitation of the  $\text{BaCO}_3$ .

<sup>2</sup>  $\text{NaCN}$  carrier added.

<sup>3</sup> Carriers added.

<sup>4</sup> The cleanup consisted of material recovered by a further barium precipitation of several of the solutions remaining from recovery of the various fractions.

No original assay was made of the  $\text{C}^{14}$  content of the sample so that the efficiency of recovery could not be determined. The activity of the various portions represent a total of 0.43 milli-curie of  $\text{C}^{14}$ .

Other samples of irradiated beryllium nitride were processed, for which the original  $\text{C}^{14}$  content was known. The results of these experiments are tabulated in the following tables:

#### EXAMPLE II

##### $\text{C}^{14}$ recovered from 57.95 gm. sample of irradiated $\text{Be}_3\text{N}_2$ sample

| Origin of Fraction      | Product as $\text{BaCO}_3$ , mg. | Specific Activity, c./m./mg. of $\text{BaCO}_3$ | Total $\text{C}^{14}$ , c./m. |
|-------------------------|----------------------------------|-------------------------------------------------|-------------------------------|
| $\text{CO}_2$           | 25.1                             | $4.14 \times 10^6$                              | $1.04 \times 10^7$            |
| $\text{HCN}$            | 1,971.0                          | $3.34 \times 10^5$                              | $1.33 \times 10^7$            |
| $\text{CH}_4\text{-CO}$ | 1,012.0                          | $1.51 \times 10^6$                              | $1.23 \times 10^7$            |
| Oxidizable <sup>2</sup> | 807.0                            | $5.39 \times 10^5$                              | $4.35 \times 10^6$            |
| Cleanup                 | 150.0                            | $4.57 \times 10^4$                              | $6.86 \times 10^5$            |

<sup>1</sup> The  $\text{AgCN}$  precipitate was collected on filter paper and the precipitate and paper were ignited together.

<sup>2</sup> Carriers added.

$\text{C}^{14}$  originally present \_\_\_\_\_ millicuries 12.2  
Total  $\text{C}^{14}$  recovered \_\_\_\_\_ do 11.3  
Percentage recovered \_\_\_\_\_ per cent 93

#### EXAMPLE III

##### $\text{C}^{14}$ recovered from a 57.83 gm. sample of irradiated $\text{Be}_3\text{N}_2$

| Origin of Fraction                     | Product as $\text{BaCO}_3$ , mg. | Specific Activity, c./m./mg. of $\text{BaCO}_3$ | Total $\text{C}^{14}$ , c./m. |
|----------------------------------------|----------------------------------|-------------------------------------------------|-------------------------------|
| $\text{CO}_2$                          | 135.4                            | $1.05 \times 10^6$                              | $1.42 \times 10^6$            |
| $\text{HCN}$                           | 172.2                            | $6.31 \times 10^5$                              | $8.71 \times 10^5$            |
| $\text{CH}_4\text{-CO}$                | 1,363.7                          | $1.75 \times 10^6$                              | $2.39 \times 10^6$            |
| Oxidizable <sup>1</sup> first portion  | 890.5                            | $6.18 \times 10^5$                              | $5.50 \times 10^5$            |
| Oxidizable <sup>1</sup> second portion | 148.2                            | $1.71 \times 10^5$                              | $2.53 \times 10^5$            |
| Cleanup                                | 143.0                            | $3.33 \times 10^4$                              | $4.77 \times 10^5$            |

<sup>1</sup> Carriers added.

<sup>2</sup> Additional carrier added and boiling and sweeping continued 24 hours.  
Original  $\text{C}^{14}$  content of sample \_\_\_\_\_ millicuries 19.7  
Total  $\text{C}^{14}$  recovered \_\_\_\_\_ do 18.7  
Percentage of  $\text{C}^{14}$  recovered \_\_\_\_\_ per cent 95.0

It will be noted from the foregoing examples that the process is capable of high efficiency in recovering  $\text{C}^{14}$ . It will also be noted that the various fractions vary somewhat in the specific activity values obtained. These variations are partially explainable on the basis that  $\text{Be}_3\text{N}_2$  as prepared may contain some normal carbon contamination in the form of free carbon, carbide, and other compounds. Further, in the processes for handling radioactive materials, it has been found desirable to add carriers to the reaction to facilitate handling. These extraneous carbon compounds will, of course, be collected along with the  $\text{C}^{14}$  activities. The present process does give differentiation of fractions having enhanced specific activity and is therefore in the nature of an improvement of the simpler mass collection process.

Operation of the present process has been proven very successful in eliminating the difficulties of earlier methods. As noted above, the recovery efficiency is high, the product may be obtained in highly enhanced fractions, and  $\text{C}^{14}$  is recovered in a stable and convenient form which may be utilized in synthesizing  $\text{C}^{14}$  compounds.

While it may be considered that the embodiments as disclosed are of a preferred nature, various changes may be made without departing from the invention, and it is intended to cover all such that come within the true scope and spirit of the appended claims.

What is claimed is:

1. In a method for recovering  $\text{C}^{14}$  activities contained in neutron irradiated metal nitrides, the step comprising reacting said neutron irradiated nitrides containing  $\text{C}^{14}$  activities with mineral acid, thereby releasing said activities from said nitrides.

2. The process as in claim 1, wherein said metal nitride comprises beryllium nitride and said mineral acid comprises sulfuric acid.

3. In a method for recovering  $\text{C}^{14}$  activities contained in neutron irradiated metal nitrides, the steps comprising reacting said neutron irradiated nitrides containing  $\text{C}^{14}$  activities with mineral acid and gaseously entraining  $\text{C}^{14}$  activities released by said acidic reaction.

4. The process as in claim 3, wherein said metal nitride comprises beryllium nitride and said mineral acid comprises sulfuric acid.

5. In a method for recovering  $\text{C}^{14}$  activities contained in neutron irradiated metal nitrides, the steps comprising reacting said neutron irradiated nitrides containing  $\text{C}^{14}$  activities with mineral acid, gaseously entraining  $\text{C}^{14}$  activities released by said acid reaction, and absorbing said entrained  $\text{C}^{14}$  activities.

6. The process as in claim 5, wherein said metal nitride is beryllium nitride and said mineral acid is sulfuric acid.

7. In a method for recovering  $\text{C}^{14}$  activities contained in neutron irradiated metal nitrides, the steps comprising reacting said neutron irradiated nitrides containing  $\text{C}^{14}$  activities with mineral acid, gaseously entraining  $\text{C}^{14}$  activities released by said reaction, combusting said entrained  $\text{C}^{14}$  activities, and absorbing said combusted  $\text{C}^{14}$  activities.

8. The process as in claim 7, wherein said metal nitride is beryllium nitride and said mineral acid is sulfuric acid.

9. In a method for recovering  $\text{C}^{14}$  activities contained in neutron irradiated metal nitrides, the steps comprising reacting said neutron ir-

7  
radiated nitrides containing C<sup>14</sup> activities with mineral acid, adding oxidizing agent to said reacted nitrides, gaseously entraining C<sup>14</sup> activities from said acid treating and oxidizing steps, absorbing said entrained activities, combusting unabsorbable activities, and absorbing said combusted unabsorbable activities.

10. The process as in claim 9, wherein said metal nitride is beryllium nitride and said mineral acid is sulfuric acid.

11. In a method for recovering C<sup>14</sup> activities contained in neutron irradiated metal nitrides, the steps comprising reacting said neutron irradiated nitrides containing C<sup>14</sup> activities with mineral acid, adding oxidizing agent to said reacted nitrides, gaseously entraining C<sup>14</sup> activities produced by said acid reaction and oxidation, combusting said gaseously entrained C<sup>14</sup> activities, and absorbing said combusted activities.

12. The process as in claim 11, wherein said nitride is beryllium nitride and said mineral acid is sulfuric acid, and wherein said combusted activities are absorbed in alkaline solution to form carbonates therein.

13. In a method for recovering C<sup>14</sup> activities contained in neutron irradiated metal nitrides, the steps comprising: (1) reacting said neutron irradiated nitrides containing C<sup>14</sup> activities with mineral acid, (2) oxidizing C<sup>14</sup> activities in solution, (3) vaporizing C<sup>14</sup> activities released by steps (1) and (2), (4) absorbing said C<sup>14</sup> activities vaporized in step (3), (5) combusting C<sup>14</sup> activities not absorbable in step (4), (6) absorbing said C<sup>14</sup> activities combusted in step (5), (7) precipitating insoluble carbonate from absorbate derived from step (6), (8) combusting C<sup>14</sup> activities absorbed in step (4), (9) absorbing said C<sup>14</sup> activities combusted in step (8), and (10) precipitating insoluble carbonate from absorbate derived in step (9).

14. In a process for recovering C<sup>14</sup> activities contained in neutron irradiated metal nitrides, the steps comprising: (1) reacting said neutron irradiated nitrides containing C<sup>14</sup> activities with mineral acid, (2) vaporizing C<sup>14</sup> activities from the reaction mixture of step (1), (3) absorbing C<sup>14</sup> activities vaporized in step (2) in an alkaline medium, (4) combusting C<sup>14</sup> activities unabsorbable in step (3), (5) absorbing C<sup>14</sup> activities combusted in step (4) in an alkaline medium, (6) treating

8  
the reaction mixture remaining from step (2) with solution oxidant, (7) vaporizing C<sup>14</sup> activities released in step (6), (8) combusting said C<sup>14</sup> activities vaporized in step (7), (9) absorbing said activities combusted in step (8) in an alkaline medium, (10) precipitating insoluble carbonate from the solution obtained in step (8), (11) precipitating insoluble cyanide from the solution remaining from step (10), (12) combusting 10 said insoluble cyanide obtained in step (11) absorbing in alkaline medium the combustion products produced in step (12), (13) precipitating insoluble carbonate from the solution obtained in step (12), and (14) precipitating insoluble carbonate from the absorbate derived from step (5).

15. The process as in claim 14, wherein said metal nitride comprises beryllium nitride and wherein sulfuric acid comprises the mineral acid 20 employed in step (1), chromium trioxide is the solution oxidant employed in step (6), and barium carbonate is the insoluble carbonate produced in steps (10), (13) and (14).

16. In a method for recovering C<sup>14</sup> contained 25 in neutron irradiated beryllium nitride the steps comprising: (1) reacting said neutron irradiated beryllium nitride containing C<sup>14</sup> activities with sulfuric acid to release the C<sup>14</sup> compounds contained therein, (2) oxidizing said compounds in 30 acid solution with chromium trioxide, (3) vaporizing the oxidized C<sup>14</sup> compounds from step (2), (4) absorbing in alkaline solution the C<sup>14</sup> compounds vaporized in step (3), (5) combusting C<sup>14</sup> compounds not absorbable in step (4), (6) absorbing in alkaline solution the combusted C<sup>14</sup> compounds derived from step (5), (7) precipitating insoluble carbonate from the solution derived 35 from step (6), (8) combusting the C<sup>14</sup> compounds derived in step (4), (9) absorbing in alkaline solution the C<sup>14</sup> compounds combusted in step (8), and (10) precipitating insoluble carbonates from the solution derived in step (9).

BERNARD A. FRIES.

#### REFERENCES CITED

The following references are of record in the file of this patent:

Science, vol. 105, No. 2723, pp. 265-267, March 50 7, 1947.